

## United States Patent Office

1

2,804,391

## MOTHPROOFING AND WATERPROOFING COMPOSITION

Vincent J. Keenan, Ardmore, Frank J. Gozlow, Philadelphia, and Robert B. Doan, Drexel Hill, Pa., assignors to The Atlantic Refining Company, Philadelphia, Pa., a corporation of Pennsylvania

No Drawing. Application June 15, 1954,  
Serial No. 436,975

3 Claims. (Cl. 106—15)

The present invention relates to the mothproofing and waterproofing of fabrics. In a more specific aspect the present invention relates to an improved composition for simultaneously waterproofing and mothproofing fabrics.

It has been known in the past that fabrics used for clothing and other purposes may be waterproofed by treating the fabric with an emulsion of a wax-type waterproofing agent. It is also known that fabrics may be made moth resistant by treatment with an emulsion of an insecticide such as DDT (dichloro-diphenyl-trichloroethane), etc. It would therefore appear to be highly desirable to treat a fabric with both types of treating agents to produce a fabric which is not only water resistant but moth resistant in addition. In order to accomplish this end, it has therefore been proposed that a fabric be treated with an emulsion of a waterproofing agent and an emulsion of a mothproofing agent. This proposed method comprises first treating the fabric with an aqueous emulsion of a waterproofing agent and thereafter treating the waterproofed fabric with an aqueous emulsion of a mothproofing agent. However, this process has not proven entirely satisfactory since it has been found that the application of the mothproofing emulsion has either removed part of the previously deposited waterproofing agent or increased the amount of water which the fabric will absorb and retain.

It is therefore an object of the present invention to provide an improved method composition for mothproofing and waterproofing fabrics. Another object of the present invention is to provide an improved method and composition for mothproofing a fabric which has previously been waterproofed. Another and further object of the present invention is to provide an improved method and composition for simultaneously waterproofing and mothproofing a fabric which can be conducted in a single treating bath. Still another object of the present invention is to provide an improved mothproofing composition which will not deleteriously affect the water resistant properties of the previously waterproofed fabric. Other and further objects of the present invention will be obvious to those skilled in the art in the following detailed description of this invention.

It has been found that an emulsion type mothproofing composition containing an anionic emulsifier, and more specifically an amine salt of an alkyl aryl sulfonic acid, may be applied to a fabric without deleteriously affecting the water resistant properties of the fabric. It has also been found in accordance with the present invention that fabrics may be simultaneously waterproofed and mothproofed by treating the fabric with a mixture of an emulsion of a waterproofing agent and the novel mothproofing emulsions of the present invention.

A typical emulsifiable mothproofing composition suitable for use in accordance with the present invention has the following approximate composition: 25% DDT powder, 5% emulsifier, 10% xylene. It is obvious that other emulsifiable insecticidal compounds and other solvents may be employed in the above stated composition without departing from the generic concept forming the basis

2

of the present invention. It is also obvious that slight variations in the concentrations of insecticide emulsifier and solvent may also be made. The emulsifiers heretofore used in the prior art have generally been non-ionic type emulsifiers such as polyethylene glycol alkyl aryl ethers and the like. In contrast to these non-ionic type emulsifiers, it has been found in accordance with the present invention that anionic type emulsifiers particularly amine salts of alkyl aryl sulfonic acids result in substantially improved water resistant properties when a cloth is to be treated with both mothproofing and waterproofing agents. In the application of the mothproofing concentrate to the fabric, the mothproofing concentrate is diluted with a sufficient amount of water and the fabric is treated with this solution for a time sufficient to deposit from about .3% to .5% by weight of mothproofing solids on the fabric.

A typical waterproofing concentrate suitable for use in accordance with the present invention has the following approximate composition: 67% water, 24% paraffin wax, 1% carnauba wax, 8% aluminum salt. Other wax type waterproofing agents are also suitable for use in accordance with the present invention and the concentrations of ingredients set forth in the above mentioned composition may also be varied. In the application of this waterproofing composition to a fabric, the waterproofing concentrate is diluted with water and the fabric is immersed in the resultant solution for a time sufficient to deposit from about 0.6 to 1.0% by weight of waterproofing solids on the fabric.

Where a fabric is to be both mothproofed and waterproofed, it is generally desirable to employ the mothproofing concentrate and the waterproofing concentrate in the ratio of about 1:2. It has been found that the most economical treatment is provided when the minimum amount of insecticide required to give satisfactory mothproofing is employed and double that percentage of waterproofing agent is used. For example it has been found that concentrations of .3% mothproofing agent and .6% of waterproofing agent gave water repellency values identical to .5% of mothproofing agent and 1% of waterproofing agent. In fact, even increasing the composition to include 2% of mothproofing agent and 4% of waterproofing agent served only to raise the water repellency of the treated fabric by 5%.

In order to illustrate the advantages of the novel mothproofing composition of the present invention, the following examples are given:

## EXAMPLE I

Two batches of a mothproofing composition were prepared by mixing 25% of DDT powder with 70% of xylene and 5% of an emulsifier. One of these batches contained an amine salt of a sulfonic acid as the emulsifier and will be designated herein as the anionic concentrate while the other batch contained a non-ionic emulsifier which is a polyethylene glycol alkyl aryl ether and is available commercially as Triton X-100. These mothproofing concentrates were then mixed with equal volumes of water and agitated to form a creamy emulsion. The emulsified mothproofing concentrates were then added to a bath containing a waterproofing concentrate composed of 67% water, 24% paraffin wax, 1% carnauba, and 8% of an aluminum salt and the baths were diluted with water to produce the treating solutions shown in Table I below. In addition to these treating baths, the third treating bath was prepared by dissolving 4% of the waterproofing concentrate in water.

3 inch by 3 inch test samples were cut from a bolt of 18 ounce wool serge. The test samples were then immersed in a bath and gently worked for 1 minute. The samples were then removed and passed once through a

wringer after which they were immediately weighed. The percent pick-up shown in Table I is calculated by subtracting the wet weight of the sample from the dry weight of the sample and dividing this difference by the dry weight of the sample and multiplying by 100. The samples were then cured at a temperature of 300° F. for 6 minutes and allowed to condition at room temperature and humidity for at least 4 hours before reweighing. This weight was recorded as the cured weight. The samples were then subjected to the "immersion absorption test." This test is described in detail in Federal Specification CCC-T-191a Supplement, October 8, 1945, for textiles, general specifications, test methods, part III, 5b (2). Summarily this test is a measure of the weight percent of water, based upon the weight of the original sample, which is absorbed by the treated textile fabric when immersed in water. In order for a waterproofed and mothproofed fabric to be acceptable when subjected to the immersion absorption test, the percent water pick-up or percent rewetting should be not greater than the rewetting percentage of the untreated fabric. Therefore, an untreated sample of the same fabric employed in the other tests was also subjected to the immersion absorption test for comparative purposes and the results of these tests are shown in Table I.

It is to be observed from Table I that the rewetting percentage for the samples treated with the anionic containing emulsifier of the present invention did not exceed 39.4% and was below the rewetting percentage for the untreated samples. On the other hand, the fabrics treated with the solution containing the non-ionic emulsifier was at least twice that obtained for the materials treated in accordance with the present invention and nearly twice that of the untreated fabric. It is also to be observed that the materials treated in accordance with the present invention have a rewetting percentage equivalent to that obtained for a sample treated with waterproofing agent alone containing no mothproofing ingredients.

In addition to the data reported on Table I, it was also noted that the fabrics treated in accordance with the present invention had a substantially improved appearance over those treated with a solution containing the non-ionic emulsifier. The samples treated with the solution containing the non-ionic emulsifier had a harsher and more wiry appearance than the samples treated with the solution containing the anionic emulsifiers of the present invention.

## EXAMPLE II

In order to further illustrate the advantages of the composition of the present invention, a second series of tests were made in which solutions were prepared as outlined in Example I. A cloth was passed through the treating solution continuously. The results obtained while continuously treating the cloth with a solution containing the non-ionic emulsifier are given in Table II below.

It is to be observed from Table II that the rewetting pick-up decreased with the passage of successive samples through the bath containing the non-ionic emulsifier. Although these results would at first blush indicate that this treating solution improved during use, there are various disadvantages connected with this change during successive treatment. In the first instance, this change would make it extremely difficult to obtain uniform results in a continuous treating process. In addition, it was noted that the fabric appeared to have a natural affinity for the non-ionic type emulsifiers and as a result the bath was continuously being depleted of emulsifier and eventually the emulsion exhibited a tendency to break. This breaking of the emulsion results in the deposition of a white deposit of DDT powder on the fabric. On the other hand, materials treated with a solution containing the anionic emulsifier of the present invention gave consistent rewetting percentages throughout and there was no evidence of the deposition of powdered DDT on the fabric.

Table I

| Treating Solution             | Impregnation  |                       |                   |               |                |                        | Re-Wet Test         |                   |               |                |                        |
|-------------------------------|---------------|-----------------------|-------------------|---------------|----------------|------------------------|---------------------|-------------------|---------------|----------------|------------------------|
|                               | Sample Number | Initial Weight, Grams | Wet Weight, Grams | Pickup, Grams | Percent Pickup | Average Percent Pickup | Cured Weight, Grams | Wet Weight, Grams | Pickup, Grams | Percent Pickup | Average Percent Pickup |
| 0.5% Mothproofing Conc.       | 1             | 2.6                   | 4.5               | 1.9           | 73.1           |                        | 2.5173              | 3.3280            | 0.8107        | 32.2           |                        |
| 1.0% Waterproofing Conc.      | 2             | 2.9                   | 4.7               | 1.8           | 62.1           | 73.5                   | 2.6614              | 3.4510            | 0.7896        | 29.7           | 31.8                   |
| Anionic Emulsifier            | 3             | 2.1                   | 4.1               | 2.0           | 95.4           |                        | 2.5526              | 3.4080            | 0.8554        | 33.5           |                        |
| 0.834% Mothproofing Conc.     | 4             | 2.7                   | 4.5               | 1.8           | 66.7           |                        | 2.6833              | 3.5920            | 0.9087        | 33.8           |                        |
| 1.668% Waterproofing Conc.    | 5             | 2.9                   | 4.7               | 1.8           | 62.0           | 61.3                   | 2.7142              | 3.5430            | 0.8238        | 30.6           | 31.7                   |
| Anionic Emulsifier            | 6             | 2.9                   | 4.5               | 1.6           | 55.2           |                        | 2.7339              | 3.5690            | 0.8351        | 30.6           |                        |
| 0.5% Mothproofing Conc.       | 7             | 2.0088                | 4.3200            | 1.4112        | 48.5           |                        | 2.9184              | 3.8970            | 0.9786        | 33.5           |                        |
| 1.0% Waterproofing Conc.      | 8             | 2.9426                | 4.5080            | 1.5654        | 53.2           | 50.8                   | 2.9592              | 3.8210            | 0.8618        | 29.1           | 30.9                   |
| Anionic Emulsifier            | 9             | 2.8611                | 4.3095            | 1.4384        | 50.6           |                        | 2.8713              | 3.7370            | 0.8657        | 30.2           |                        |
| 4.0% Waterproofing Conc. Only | 10            | 2.2903                | 2.8820            | 0.5917        | 25.8           |                        | 2.2021              | 2.8180            | 0.6159        | 29.4           |                        |
|                               | 11            | 2.2496                | 2.7720            | 0.5224        | 23.3           | 24.2                   | 2.1600              | 2.8930            | 0.7330        | 33.9           | 30.8                   |
|                               | 12            | 2.2417                | 2.7710            | 0.5293        | 23.6           |                        | 2.1529              | 2.7770            | 0.6241        | 29.0           |                        |
| 0.5% Mothproofing Conc.       | 13            | 2.1944                | 3.3940            | 1.1999        | 54.8           |                        | 2.1470              | 2.9945            | 0.8466        | 39.4           |                        |
| 1.0% Waterproofing Conc.      | 14            | 2.2370                | 3.4340            | 1.1970        | 53.6           | 55.9                   | 2.1837              | 2.9803            | 0.7468        | 34.2           | 35.8                   |
| Anionic Emulsifier            | 15            | 2.2402                | 3.3440            | 1.1038        | 49.2           |                        | 2.1748              | 2.9075            | 0.7327        | 33.7           |                        |
| 0.5% Mothproofing Conc.       | 16            | 2.2993                | 4.0690            | 1.7397        | 76.5           |                        | 2.3133              | 4.0860            | 1.7727        | 75.6           |                        |
| 1.0% Waterproofing Conc.      | 17            | 2.2661                | 3.9230            | 1.6569        | 73.1           | 76.0                   | 2.2746              | 4.0040            | 1.7294        | 76.3           | 75.8                   |
| Non-Ionic Emulsifier          | 18            | 2.2810                | 4.0660            | 1.7850        | 78.5           |                        | 2.2671              | 3.9750            | 1.7079        | 75.5           |                        |
| Untreated                     | 19            | 2.2785                |                   |               |                |                        | 2.2785              | 3.2690            | 0.9905        | 43.5           |                        |
|                               | 20            | 2.2086                |                   |               |                |                        | 2.2086              | 3.0935            | 0.8849        | 40.1           | 42.4                   |
|                               | 21            | 2.1879                |                   |               |                |                        | 2.1879              | 3.1450            | 0.9571        | 43.7           |                        |

Table II

| Treating Solution        | Impregnation  |                       |                   |               |                |                        | Re-Wet Test         |                   |               |                |                        |
|--------------------------|---------------|-----------------------|-------------------|---------------|----------------|------------------------|---------------------|-------------------|---------------|----------------|------------------------|
|                          | Sample Number | Initial Weight, Grams | Wet Weight, Grams | Pickup, Grams | Percent Pickup | Average Percent Pickup | Cured Weight, Grams | Wet Weight, Grams | Pickup, Grams | Percent Pickup | Average Percent Pickup |
| 0.5% Mothproofing Conc.  | 1             | 2.5653                | 4.6710            | 2.1057        | 82.1           |                        | 2.4942              | 4.4630            | 1.9688        | 79.1           |                        |
| 1.0% Waterproofing Conc. | 2             | 2.5614                | 4.5720            | 2.0106        | 78.5           | 80.1                   | 2.4974              | 4.3150            | 1.8176        | 72.8           | 66.4                   |
| Non-Ionic Emulsifier     | 3             | 2.6751                | 4.7305            | 2.0554        | 77.0           |                        | 2.6012              | 4.3380            | 1.7368        | 67.0           |                        |
|                          | 4             | 2.6424                | 4.8260            | 2.1836        | 82.6           |                        | 2.5675              | 3.7640            | 1.1965        | 46.6           |                        |

5  
EXAMPLE III

In order to demonstrate the stability of the treating baths prepared in accordance with the present invention four treating solutions were made up. Two of these solutions contained 96 gram of water, 2 grams of waterproofing concentrate and 2 grams of the mothproofing agent of the present invention. The other two samples contained 92 grams of water, 4 grams of waterproofing agent and 4 grams of mothproofing agent. These treating solutions were permitted to stand over night and were then observed on the following day. The two baths containing 2 grams each of waterproofing concentrate and mothproofing concentrate were in good condition after standing. The other two baths containing larger amounts of mothproofing agent and water proofing agent showed a slight break of the emulsion over night with slight oil separation. However, no solids were precipitated out and the solution could be easily reemulsified by stirring. In addition to these tests, further tests were conducted in which treating baths prepared in accordance with the present invention were permitted to stand over night and samples of fabric were treated with these baths the following morning. The samples treated in accordance with this experiment showed a rewetting percentage of about 30.9% and there was no evidence of a white deposit on the treated samples.

We claim:

1. An improved mothproofing and waterproofing composition for treating fabrics consisting essentially of an aqueous emulsion containing small amounts of a mixture

## 6

of a mothproofing concentrate consisting of about 25 percent by weight of dichloro-diphenyl-trichloroethane, 70 percent of xylene, and 5 percent of an anionic emulsifier consisting essentially of an amine salt of an alkyl aryl sulfonic acid and a waterproofing composition consisting of about 67 percent of water, 24 percent of paraffin wax, 1 percent carnauba wax, and 8 percent of an aluminum salt.

2. A composition in accordance with claim 1 wherein 10 the mothproofing composition and the waterproofing composition are present in a ratio of about 1:2.

3. A composition in accordance with claim 1 wherein 15 the mothproofing composition is present in an amount of about 0.5% by weight of the total emulsion and the waterproofing composition is present in an amount of about 1% by weight of the total emulsion.

## References Cited in the file of this patent

## UNITED STATES PATENTS

|    |           |              |       |               |
|----|-----------|--------------|-------|---------------|
| 20 | 2,369,992 | Treacy       | ----- | Feb. 20, 1945 |
|    | 2,402,351 | Smith et al. | ----- | June 18, 1946 |
|    | 2,448,910 | Reamer       | ----- | Sept. 7, 1948 |
|    | 2,456,595 | Road         | ----- | Dec. 14, 1948 |
| 25 | 2,556,300 | Showalter    | ----- | June 12, 1951 |
|    | 2,635,055 | Figdor       | ----- | Apr. 14, 1953 |

## OTHER REFERENCES

"Soap and Sanitary Chemicals," of December 1947, page 171; 106-15 A. F. Atlas "Surface Active Agents," 30 Atlas Powder Co. (1948), page 49.